

Dec. 7, 1954

R. O'HALLORAN

2,696,471

CARBON BLACK LUBRICATING GREASE

Filed Dec. 10, 1952

2 Sheets-Sheet 1

FIG. - 1



Rosemary O'Halloran Inventor

By Elwin M. Thuma Attorney

Dec. 7, 1954

R. O'HALLORAN

2,696,471

CARBON BLACK LUBRICATING GREASE

Filed Dec. 10, 1952

2 Sheets-Sheet 2

FIG. - 2



Rosemary O'Halloran Inventor

Big Law, Inc. Attorneys

# United States Patent Office

2,696,471

Patented Dec. 7, 1954

1

2,696,471

## CARBON BLACK LUBRICATING GREASE

Rosemary O'Halloran, Roselle Park, N. J., assignor to Standard Oil Development Company, a corporation of Delaware

Application December 10, 1952, Serial No. 325,092

8 Claims. (Cl. 252—22)

The present invention relates to an improved lubricating grease composition and particularly to a carbon black-aluminum soap grease which is suitable for use in heavy industrial equipment such as steel roller mills and the like where high temperatures and heavy unit pressure conditions are encountered.

It has been suggested previously in application Serial No. 218,260 filed March 29, 1951, now Patent No. 2,653,131, by the present inventor that a combination of aluminum soap and carbon black as thickening agents in lubricating oil results in the formation of a superior grease for heavy industrial applications of the type mentioned above. According to the present invention it has been found that greases of improved yield and other advantageous properties may be obtained by substituting an acid treated mineral base lubricating oil for the usual black oil employed in greases of this type and that further improvement may be obtained by using a small percentage of saturated fatty acid of the C<sub>14</sub> to C<sub>20</sub> range in combination with the soap and carbon black.

It has been known in the prior art to use extreme pressure agents in heavy duty lubricating greases of the type under consideration. Commonly a sulfurized fatty oil and other extreme pressure additives, which may include oleic acid in some cases, have been added to lubricating greases of the carbon black type for some operations. It has now been discovered, however, that a very substantial increase in consistency is obtained by combining an acid treated oil with the carbon black and

2

is between 5 and 25%, preferably about 10 to 12%, and may be either acetylene carbon black or channel black or a mixture thereof. For optimum extreme pressure properties, however, channel black or at least a substantial proportion of channel black with some acetylene black is preferable. The saturated fatty acid, which replaces the oleic acid of some types of prior art grease compositions, is used in proportions of 0.5 to 4%, preferably about 2%, and the sulfurized fatty oil which forms the principal extreme pressure agent is used in proportions of 5 to 15%, preferably about 8 to 10%. Also, it is desirable that tri-ester of phosphoric acid, such as tricresyl phosphate or tributyl phosphate, be used in proportions of 0.5 to 2%, preferably about 1%. Tricresyl phosphate ordinarily is preferred over tributyl phosphate for this purpose.

A series of tests were made using various combinations of mineral oil base and varying proportions of a channel type carbon black of fine particle size sold under the trade name "Superba Black." Each of the compositions contained about 9% of sulfurized sperm oil although proportions of 5 to 15% of sulfurized sperm oil or other sulfurized or phospho-sulfurized fatty oils such as lard oil, cotton seed oil and the like can be employed with reasonably satisfactory results.

In each case a standard commercial aluminum stearate previously prepared was used as the soap ingredient of the thickener and in some cases 2% of the hydrogenated fish oil acids mentioned above were employed. The others contained 2% of oleic acid. An additional ingredient, tricresyl phosphate in proportions of 1%, was added in each composition. All percentages given are by weight, based on the total composition. The greases described herein were all made by the cold blending procedure described in the parent application, Serial No. 218,260, mentioned above.

It will be noted from the table below that the greases containing the saturated fatty acid all had a dropping point above 500° F. The results of these several experiments are indicated in Table I. The pressure oil separation test referred to consists of collecting and weighing the oil expressed from a 50 g. grease sample through double No. 0 filter paper after 20 hours under 100 p. s. i. g. N<sub>2</sub> pressure in a metal cylinder.

TABLE I  
Experimental steel mill greases containing 9% sulf. sperm  
oil, 2% oleic acid, 1% tricresyl phosphate

|      | Soap Solution                                                         | Mineral Oil Base                            | "Superba Black,"<br>Percent | Prep.<br>Scale | Dropping<br>Point,<br>° F. | Worked<br>Pen.,<br>mm./10 | Pressure<br>Oil Sep.,<br>Percent | Timken<br>Test |
|------|-----------------------------------------------------------------------|---------------------------------------------|-----------------------------|----------------|----------------------------|---------------------------|----------------------------------|----------------|
| I    | 2.8% Commercial Aluminum Stearate                                     | Crude Distillate Oil                        | 10                          | Lab            | 468                        | 405                       | 1.0-3.2                          | Pass 38.       |
| II   | do                                                                    | do                                          | 10                          | Pilot          | 431                        | 445                       | 1.0                              |                |
| III  | do                                                                    | do                                          | 12                          | Lab            |                            | 385                       |                                  |                |
| IV   | do                                                                    | Acid Treated Oil, 70<br>S. S. U. at 210° F. | 10                          | Lab            |                            | 375                       |                                  |                |
| V    | 2.8% Commercial Al. Stearate+2.0% Hy-<br>drofol Acid 53. <sup>1</sup> | do                                          | 10                          | Lab            | 500+                       | 343                       | 2.8                              | Pass 38.       |
| VI   | do <sup>1</sup>                                                       | do                                          | 2 10                        | Lab            | 500+                       | 300                       | 2.0                              | Fail 33.       |
| VII  | do <sup>1</sup>                                                       | do                                          | 10                          | Pilot          | 500+                       | 321                       | 3.2                              | Pass 38.       |
| VIII | do <sup>1</sup>                                                       | do                                          | 2 5                         | do             | 500+                       | 340                       | 1.6                              | Pass 33.       |
| IX   | Commercial Acetylene Black EP Grease<br>Desired Level of Performance  |                                             |                             |                | 500+                       | 361                       | 8.6                              | Fail 33.       |
|      |                                                                       |                                             |                             |                | 500+                       | 380 Max                   | 5.0 Max                          | Pass 33.       |

<sup>1</sup> Contains no oleic acid.

<sup>2</sup> 10% acetylene black.

<sup>3</sup> 5% "Superba" (channel) black plus 5% acetylene black.

aluminum soap thickeners and a further and substantial improvement is obtained by incorporating saturated fatty acids of the C<sub>14</sub> to C<sub>20</sub> range. For example, fatty acids sold commercially under the trade names "Hydrofol Acids 53" and "Hydrofol Acids 54" are used in the extreme pressure component, replacing oleic acid where the latter has previously been employed.

Hence the composition of the present invention comprises a major proportion of acid treated petroleum base lubricating oil containing between 1 and 5% by weight of aluminum soap of predominantly saturated fatty acids of the C<sub>12</sub> to C<sub>22</sub> range. The preferred aluminum soap is aluminum stearate and it is preferably used in proportions of about 2 to 3%. The carbon black content

70 It will be noted from the above table that when the saturated fatty acids and the acid treated oil were used to replace oleic acid and the crude distillate oil, respectively, the penetration improved from 405 mm./10 in a laboratory batch to 343 mm./10 other ingredients and processing being the same. In a pilot plant batch of grease the penetration value of the grease containing the "Hydrofol" (saturated) acids was only 321 mm./10. The difference represents a considerable increase in yield value. Definite improvement was obtained by substituting the saturated fatty acid for the oleic acid in the laboratory product also (compare V and VII of Table I). The substitution of saturated for unsaturated fatty acids brought the worked penetration in the standard ASTM

test apparatus from 375 mm./10 down to 343 mm./10 with the same acid treated base oil.

Inasmuch as the cost of the soap and carbon thickeners for these heavy industrial greases is a very substantial item in their production it is apparent that substantial savings may result from the substitution of acid treated oil for conventional black oil, because of the improved yields mentioned above. Even greater savings result when the saturated fatty acids are employed in place of the conventional oleic acid. A combination of these features results in very substantial improvements in yield without any sacrifice in quality.

Greases containing both oleic acid and saturated fatty acids were tested also for extreme pressure performance. Both of them carried a load of 38 pounds in the standard Timken test machine. This is regarded as entirely satisfactory. The commercial grease listed in Example IX of Table I did not carry even 33 pounds which is considered minimum for satisfactory performance. It had a worked penetration of 361 mm./10 which is acceptable although rather soft, but its oil separation was excessive, 8.6% as compared with 2.8% and 3.2%, respectively, for the laboratory and pilot plant batches of the present invention. As noted in the table a maximum amount of oil separation of 5% is acceptable. The use of straight channel black (Ex. I, V, VII) results in superior Timken machine performance as shown in the table. However, the high temperature properties of this blend, as shown by high temperature pressure viscometer runs, are not equivalent to those where at least a part of the channel black is replaced by acetylene black. These runs are shown graphically in the drawing, Figure 1. It may be seen on the figure that Ex. VIII, the grease of invention (containing 50-50 channel and acetylene black) is equivalent in bodying properties to straight acetylene black grease (Ex. VI) and far superior to straight channel (Ex. VII). Reference to the table will show that the extreme pressure performance of Ex. VIII is satisfactory, showing a Timken pass at 38.

Extreme pressure properties of the grease of the invention are also shown by its performance in the 4-ball wear test. This test was developed by the United States Navy and has been described in various references. The performance standards have been set up by Aluminum Co. of America and published in their ML-792 (Revised April, 1951) Specification covering a multipurpose extreme pressure grease. The grease of the present invention is compared with a typical grease meeting this specification below:

|                | Example VIII | Commercial Alcoa ML-792 Grease | ML-792 Spec. |
|----------------|--------------|--------------------------------|--------------|
| E. P. Value    | 38           | 23                             | 21 min.      |
| Weld Point, kg | 316          | 140                            | 125 min.     |

Complete load versus wear-spot curves for these two greases are plotted in Figure 2.

It will be understood that various modifications may be made in process and product without departing from the spirit of the invention. The method used for preparing the greases described above was to add the fatty acids directly to aluminum soap in oil (soap concentrate or grease base), heat until fluid (250-300° F.), pan cool to ambient temperature and thereafter to stir in the carbon black, followed by adding the sulfurized sperm oil and the other extreme pressure ingredients.

What is claimed is:

1. A lubricating grease composition comprising a major proportion of acid treated petroleum base lubricating oil, 1 to 5% by weight, based on the total composition, of aluminum soap of predominantly saturated fatty acids of the C<sub>12</sub> to C<sub>22</sub> range, 5 to 25% of carbon black, 0.5 to 4% of saturated fatty acid of the C<sub>14</sub> to C<sub>20</sub> range, and 5 to 15% of a sulfurized fatty oil as an extreme pressure agent.
2. Composition according to claim 1 wherein the aluminum soap is aluminum stearate.
3. Composition according to claim 1 wherein the carbon black is acetylene black.
4. Composition according to claim 1 wherein the carbon black is a channel black.
5. Composition according to claim 1 where the carbon blacks are mixed acetylene black and channel black.
6. Composition according to claim 1 to which is added 0.5 to 2% of a tri-ester of phosphoric acid.
7. Composition according to claim 1 to which is added about 0.5 to 2% of tricresyl phosphate.
8. A lubricating grease composition consisting essentially of about 73 to 76% by weight of acid treated mineral base oil of 50 to 100 S. S. U. viscosity at 210° F., about 9% sulfurized sperm oil, about 2 to 3% of aluminum stearate, about 5% channel black, about 5% acetylene black, 2% saturated fatty acids of the C<sub>14</sub> to C<sub>20</sub> range, and about 1% tricresyl phosphate.

#### References Cited in the file of this patent

#### UNITED STATES PATENTS

| Number    | Name           | Date          |
|-----------|----------------|---------------|
| 2,367,355 | Kaufman et al. | Jan. 16, 1945 |
| 2,480,647 | Gurd et al.    | Aug. 30, 1949 |
| 2,487,260 | Morway         | Nov. 8, 1949  |